

June 4, 1940.

M. BROWN

2,203,253

ELECTROPLATING PROCESS

Filed Sept. 26, 1936



FIG. 3



INVENTOR  
M. BROWN

or H.G. Whitehorn

ATTORNEY

## UNITED STATES PATENT OFFICE

2,203,253

## ELECTROPLATING PROCESS

Morris Brown, La Grange, Ill., assignor to Western Electric Company, Incorporated, New York, N. Y., a corporation of New York

Application September 26, 1936, Serial No. 102,696

1 Claim. (Cl. 204—6)

This invention relates to electroplating processes, and more particularly to the manufacture of sheet metal by electrodeposition.

The manufacture of certain metal articles, such as tubes or foil, by electrodeposition processes, has been restricted by the tendency of the metal to adhere to the mandrel or mould on which it is deposited. In the production of foil by this method, the tension required to remove the foil from the mandrel has limited the minimum thickness and also the composition of the product. Coatings of grease, tin, zinc or mercury amalgam have been applied to the mandrel to overcome this difficulty but some of these expedients do not give entirely satisfactory results and all of them are further objectionable in that they require periodic replacement.

Objects of this invention are to provide improved methods and apparatus for the efficient electrodeposition of metal.

In accordance with one embodiment of the invention, apparatus is provided for the continuous manufacture of metal foil by electrodepositing the metal on a chromium coated rotating mandrel, and stripping the deposited metal from the mandrel in the form of a continuous sheet.

A complete understanding of the invention may be had from the following detailed description taken in conjunction with the appended drawing, in which

Fig. 1 is a schematic view, partly in section, of an electroplating apparatus, embodying the invention;

Fig. 2 is a section of the apparatus shown in Fig. 1, taken on the line 2—2, and

Fig. 3 is a sectional view taken on line 3—3 of Fig. 2.

Referring now to the drawing, a conventional continuous electroplating installation comprises a cylindrical drum or mandrel 10 which is rotatably mounted on a shaft 11 over a tank or container 12. The tank is lined with lead 13 and contains an electrolyte 14 of suitable metal salt in which the mandrel is partially immersed. In accordance with well known practises, plating current of suitable characteristics is supplied from a battery 15 or other source with its negative terminal 16 connected to the mandrel or cathode through a sliding contactor 11 engaging a conductor 18 which is imbedded in insulation in the mandrel shaft and connected to the mandrel through a wire 19. The positive terminal 20 of the battery is connected directly to the lead sheet lining of the tank which serves as an insoluble anode.

The electrolyte is circulated through the tank against the rotating mandrel by a pump or other suitable means (not shown). The tank has a rounded bottom approximately conforming with the mandrel contour. Depleted electrolyte is withdrawn from one end of the tank, replenished with metal salt in an external apparatus, (not shown) and recirculated. The metal deposited on the rotating mandrel is stripped from the mandrel surface in the form of a continuous sheet 10 or foil 21 by a revolving takeup spool 22 supported in bearings 23 over the mandrel and driven through a belt 24 by suitable and conventional mechanism (not shown) for applying a constant tension to the foil.

The general features of the apparatus and process so far described are old and well known and this invention is directed primarily to the construction of the mandrel on which the metal is deposited. The preferred construction is particularly suitable for the production of copper foil under .0003" thick which is useful in the manufacture of condensers and other products. Foil used for this purpose must be uniform in thickness and preferably has a smooth, continuous surface.

It is possible to control the thickness of the deposited sheet in general by regulation and coordination of the plating current, electrolyte composition, mandrel size and operating speed. However, copper in this dimension possesses little tensile strength and even very slight tendency of the foil to adhere to the mandrel results in breakage. It is undesirable to use temporary coatings of foreign substances on the mandrel surface to reduce sticking of the foil because the deposited metal conforms rigidly to the contour of the mandrel and reproduces any surface irregularities. It is difficult to apply these coatings smoothly and their repeated use may destroy the surface on the mandrel.

To overcome these objections, the mandrel is provided with a permanently smooth, uniform surface from which the deposited metal can be readily removed. The mandrel comprises a steel cylinder 25 (Figs. 2 and 3) which is formed to shape and ground on the outside surface to remove all irregularities and imperfections. Other materials can be used for this member, but steel is preferred because of its stability in retaining the surface and shape produced in the grinding operation. A layer of nickel 26 is plated uniformly on the ground surface of the cylinder and subsequently buffed to a high polish. A nickel coating .0005" thick is satisfactory for most in-

stallations, but this dimension can be varied rather widely, depending upon the composition of the cylinder, size of the installation, and service requirements. A uniform layer of chromium 5 27 is plated over the nickel and buffed to a high polish. This coating may also vary in thickness, but coatings around .00005" thick give good results.

The composite mandrel cylinder is supported 10 at each end by a disk shaped member 28 made of wood, fiber, or other insulating material and secured to the mandrel shaft. At each end of the mandrel cylinder, a ring 30 made of rubber or other insulating material is imbedded in the periphery of the disk. The ring projects above the surface of the mandrel to form the deposited foil with uniform, unbroken edges.

The side of the foil next to the mandrel has a smooth surface, determined by the finish on the 20 mandrel, but the other side may be spongy or rough. To smooth this outer surface, a roller 31 is rotatably mounted parallel to the mandrel in bearings 32 in contact with the foil on the mandrel surface. The roller is driven from the mandrel shaft through a twisted belt 33 engaging pulleys on the mandrel and roller shafts. The pulleys are selected to rotate the roller at a surface speed approximately 15% higher than the surface speed of the mandrel which produces a 25 burnishing action and imparts a smooth polished surface to the foil. The relative surface speeds of the roller and mandrel may be varied for different foil thicknesses and compositions and under various conditions the roller may operate at 30 speeds from 10% to 25% higher than the mandrel. The position of the burnishing roll is made adjustable relative to the mandrel by any suitable means (not shown) and the roll is located to control the final thickness dimension of the foil. 35

In the operation of the process, the chromium, being passive, prevents adherence between the foil and mandrel. As a result the foil is readily removed with a slight takeup tension which pre- 40

vents damage to the product and facilitates the manufacture of thinner foil. It is also possible with this apparatus to produce foil from materials having relatively low tensile strengths, such as gold or nickel. 5

A mandrel constructed in accordance with the above description is also suitable for the manufacture of tubes or shapes. In this process, the metal is plated on the mandrel, which may be stationary or rotating, after which the mandrel 10 is readily withdrawn from the completed article.

If desired, the chromium can be plated directly on the steel cylinder to provide a mandrel with a passive surface that will not adhere to the deposited metal. However, the intermediate layer of 15 nickel is beneficial as it facilitates the application of the chromium and the development of a smooth uniform surface. A mandrel formed entirely of chromium will operate satisfactorily, but the composite mandrel is more serviceable and 20 less costly.

Other adaptations and modifications of the specific embodiment above described are feasible and it is to be understood that the invention is limited only by the scope of the appended claim. 25

What is claimed is:

A method of producing thin copper foil which comprises electrodepositing a copper layer less than .0003" in thickness on a chromium surface while said surface is moving at a predetermined 30 speed, compressing the deposited copper against the chromium surface by means of a cylinder having a metallic surface maintained a fixed distance from the chromium surface to size the copper into foil of a predetermined thickness, 35 withdrawing the foil from the chromium surface with a predetermined tension around an arc of said cylinder, and rotating the cylinder at a surface speed from 10% to 25% higher than the speed of the chromium surface to polish the foil in the arc of contact with said cylinder. 40

MORRIS BROWN.